# EUROPEAN PATENT SPECIFICATION

(11) **EP 2 191 067 B1**
(45) Date of publication and mention of the grant of the patent: **20.06.2012**
(21) Application number: 08803525.8
(22) Date of filing: 02.09.2008
(51) Int. Cl.: D21H 13/20, D21H 13/26

(54) **PAPER COMPRISING POLYBENZAZOLE OR PRECURSOR THEREOF**
PAPIER MIT POLYBENZAZOL ODER EINEM VORLÄUFER DAVON
PAPIER CONTENANT DU POLYBENZAZOLE OU UN PRÉCURSEUR DE CE DERNIER

(30) Priority: 12.09.2007 EP 07017825
(43) Date of publication of application: 02.06.2010
(73) Proprietor: Teijin Aramid B.V., 6824 BM Arnhem (NL)
(72) Inventor: LOPEZ LORENZO, Monica, NL-6846 HN Arnhem (NL); DE WEIJER, Anton Peter, NL-6525 PN Nijmegen (NL); VISSER, Richard, NL-6824 DC Arnhem (NL)
(74) Representative: Heimann, Anette
(86) International application number: PCT/EP2008/061554
(87) International publication number: WO 2009/033983

(56) References cited:
- WO-A-2007/074368
- WO-A-2007/075575
- WO-A-2007/076332
- JP-A- 10 096 175
- JP-A- 2001 248 091
- JP-A- 2007 063 399
- US-A1- 2007 144 696
- US-B2- 6 890 636

## Description

The invention relates to a paper comprising at least one of a fiber, pulp, fibril, floc, and fibrid containing a polybenzazole structure or a polybenzazole precursor structure. The invention further pertains to a method for making such papers and to the use thereof.

It has been described in EP 07008742 that fiber, pulp, fibril, or fibrid having superior properties, including mechanical properties, can be obtained by a process in which an optical anisotropic dope, containing a high concentration of a high molecular weight aromatic polyamide having a substituent such as a hydroxy, thiohydroxy, or amine group in an acidic solvent, is applied using a wet air gap spinning process, a jet spinning process, or any other conventional method to obtain a fiber, pulp, fibril, or fibrid, which are then heat treated.

The present invention relates to paper comprising at least one of a fiber, pulp, fibril, floc, and fibrid having a polybenzazole structure with a repeating unit of formula (I) and/or (II) or its precursor structure with a repeating unit of formula (III): wherein Ar¹ and Ar² are independently a para or meta aromatic group having 4 to 12 carbon atoms, X and Y are the same or different and selected from O, S, and NH; and n is 0 or 1, and wherein the paper is free or essentially free of non-extractable phosphorus compound.
wherein the paper contains less than 0.15 wt% of non-extractable phosphorus compound.

Papers made of fibers having a polybenzazole structure are known in the art, for instance from JP 10 096175, JP 2001 248091, and WO 2007/076332.

JP 10 096175 relates to non-woven sheets rather than to paper. Furthermore, these sheets and papers have been made from fibers that are spun from polyphosphorus spinning dopes. Therefore, these papers contain a considerable amount of non-extractable phosphorus compound, since even the most sophisticated methods for removing polyphosphorus acid leaves at least 0.25 wt%. Normal commercial procedures leave about 0.4 wt% of polyphosphorus acid in the fiber (see for instance, Hu X.B. and Lesser A.J.; Abstracts of Papers of the American Chemical Society 2004, 227:U562-U562).

The terms "para" and "meta" relate to the positions of the two amino groups or the two carbonyl groups at the aromatic ring. If Ar¹ and/or Ar² contain annelated aromatic rings there are formally no para and meta positions, but the corresponding positions are called pseudo-para and pseudo-meta positions, which are included in the definition of "para" and "meta".

The paper is free or essentially free of non-extractable phosphorus compound, which means that the paper contains less than 0.15 wt% of non-extractable phosphorus compound and preferably no non-extractable phosphorus compound at all.

The present fibers, pulp, fibrils, floc, or fibrids are manufactured by a method comprising the steps of spinning or extruding a dope and solidifying it to a coagulation liquid, and then subjecting the obtained fiber as was described in EP 07008742.

The invention also relates to a precursor paper, which as such has excellent properties and therefore can be used as such. This precursor paper contains a polybenzazole precursor having the repeating unit expressed by formula (III): wherein Ar¹ and Ar² are independently an aromatic group having 4 to 12 carbon atoms, Ar¹ and Ar² have the para or meta configuration, X and Y are the same or different and selected from O, S, and NH, and n is 0 or 1.

Examples of Ar¹ are phenylene, naphthalenediyl, and bivalent heteroaromatic groups. Ar¹ may be substituted with hydroxy and/or halogen groups.

Ar¹ is preferably selected from and Ar² is a tri- or quadrivalent aromatic group with 4-12 carbon atoms. Examples of Ar² are benzenetri- or tetrayl, naphthalenetri- or tetrayl, diphenyltri- or tetrayl, and tri- or quadrivalent heterocyclic group can be listed as Ar². These Ar² moieties may be substituted with a hydroxy and/or halogen group.

Ar² is preferably selected from:

The benzene group is the most preferred Ar² group.

In a preferred embodiment Ar¹ is para- or meta-phenylene: and Ar² is wherein X and Y are O, and the straight lines represent a bond.

In addition to the above polybenzazole the fiber may also be a copolymer containing repeating units expressed by formula (IV)

In formula (III), the Ar¹ groups have independently the previously given meanings. The preferred Ar¹ group is para-or meta-phenylene.

The polybenzazole preferably comprises 40 to 100 mole% of the repeating unit expressed by formula (I) and/or (II) with 60 to 0 mole% of the repeating unit expressed by formula (IV), to a total of 100 mole%.

The polybenzazole more preferably comprises 60 to 100 mole% of the repeating unit expressed by formula (I) and/or (II) with 40 to 0 mole% of the repeating unit expressed by formula (IV), to a total of 100 mole%.

Since X is an oxygen atom (-O-), sulfur atom (-S-), or imino group (-NH-), the polybenzazole which can be obtained form the polymer precursors contains imidazole, thiazole, and/or oxazole rings.

The polybenzazole precursor containing one or more of the following repeating units is especially preferred. or or or or or

Methods for making these polymers, and for making fiber, pulp, fibril, floc or fibrid thereof are disclosed in European patent application no. EP 07008742.

Although PBO paper is known in the art, i.e. as mentioned in patent US 6890636, such paper inherently contains substantial amounts of phosphoric acid which was used as spin dope for making fiber, and which cannot completely be removed. The PBO paper of this invention contains less than 0.15 wt% of non-extractable phosphorus compound (i.e. mainly phosphoric acid), preferably much less such as less than 30 ppm, and most preferably none or virtually none of phosphorus compound (when the spin dope does not contain any phosphoric acid). Because it is known that traces of phosphoric acid may decompose PBO fibrous materials, leading to substantial loss of paper strength, it may be of utmost importance to make PBO paper that is free or at least substantially free of phosphoric acid, if such paper should maintain its strengths for long periods. The unique method for making the PBO paper of this invention resides in a method wherein the ring-closed PBO structure is obtained from an open precursor structure still having OH, SH, or NH₂ groups. These hydrophilic groups allow the precursor to dissolve in hydrophilic solvents such as water, alcohol, water-alcohol mixtures, and the like. Whereas PBO can practically only be dissolved in phosphoric acid-containing spin dopes, the present precursors can form spin dopes in said hydrophilic solvents, without using any phosphoric acid. Such spin dopes will lead to fiber, pulp, fibril, floc or fibrid that is completely or virtually completely free from phosphorus compound. PBO paper having less than 0.15 wt% phosphorus compound is unknown. The known PBO papers have been made from PBO-polyphosphorus acid-containing spin dopes, leading to paper having (much) more than 0.15 wt% non-extractable phosphorus. Although it is usually not preferred, small amounts of phosphorus acid or other phosphorus compounds can be added to the spin dope, leading to papers having minor amounts (i.e. less than 0.15 wt%) of phosphorus. The amount of phosphorus present in the paper can easily be measured by using standard methods such as by spectroscopy or titration.

The papers of this invention may include combinations of fiber, pulp, fibril, floc or fibrid, such as fibrids and floc. The papers of the invention can be made by conventional papermaking processes, which processes allow adding common additives and auxiliary materials to the material for making paper, such as pigments, binders, silicates, fillers, and other additives. The paper such obtained may be processed further such as by applying known calendaring methods to further enhance the density of the paper.

The terms "fibers, pulp, fibrils, floc, and fibrids" are well known in the field, and for instance can be found in Textile Terms and Definitions, 2nd Ed, 1955.

The term "fibrids" refers to non-granular film-like particles. The fibrids have an average length of 0.2 to 1 mm with a length-to-width aspect ratio of 5:1 to 10:1. The thickness dimension is on the order of a fraction of a micrometer. Such fibrids, when fresh, are used wet and are deposited as a binder physically entwined about the floc component of the paper. Fresh fibrids and previously-dried fibrids can be used in paper of this invention.

The term "floc" refers to short fibers, typically having a length of 2 to 12 mm and a linear density of 1-10 decitex. The floc can be fresh or it can be previously-dried. If fresh, it has not before been used in any product.

Paper pulp may comprise floc and fibrids, generally, in amounts of about 50-60%, by weight, fibrids and 40-50%, by weight, floc. Even after comminuting and milling, the floc in aramid paper pulp is bound, to some extent, by the fibrids. The fibrids, being in a dried state, are bound together or collapsed and less useful as binder material than the fresh, never-dried, fibrids; but, due to their random, rigid, irregular, shape, contribute an increased porosity to the final paper structure. For purposes of this invention, those fibrid and floc components taken from dried papers may be called previously-dried fibrids and previously-dried floc.

Dried paper sheets containing polybenzazole precursor can also be processed through a high speed milling machine, such as a turbulent air grinding mill known as a Turbomill or an Ultra-Rotor, and then wet refined. Turbulent air grinding mills are preferred for comminuting papers which have been calendered; but the grinding mills result in slightly shortened fiber lengths. Paper of this invention using paper pulp with shortened fiber lengths exhibits slightly reduced wet strength and a tendency to worsen paper machine continuity.

The paper made from the polybenzazole precursor material can be used as such. It has excellent properties as will further be demonstrated in the experimental part. However, the properties of this paper can easily be changed or improved by functionalizing at least part of the free XH and YH groups, such as OH groups. These free groups are able to react with monomers and polymers having reactive groups, such as esters, isocyanates, epoxides, and other functionalizing agents to give a covalent bond between X and/or Y and the functionalizing agent. If part of the free XH and YH groups is functionalized these papers can also be heat treated to convert the polymer precursor by a cyclizing process to ring-closed PBO polymers, thereby obtaining functionalized PBO paper.

Functionalizing of all or part of the XH and YH groups can be done in various phases of the papermaking process. Thus it is possible to functionalize (part of) the XH en YH groups in the monomer followed by polymerization with the monomer ClOOC-Ar¹-COOCl. The functionalized polymer can then be treated in any of the above described manners to obtain the paper of the invention.

Functionalizing can also be performed on the precursor polymer or the polybenzazole, as obtained by polymerization of the monomers. These polymers may contain XH and/or YH groups which can be functionalize by reaction with a functionalizing agent. The polymer can be functionalized in any of the stages during the process of making paper. Thus the polymer can be functionalized just after polymerization of the monomers, but it can also be functionalized in the form of a fiber, pulp, fibril, floc, or fibrid, or after the paper has been made. In the latter methods in most cases only the outer surface of the fiber, pulp, fibril, floc, or fibrid can easily be functionalized, which can be an advantage if only partial functionalization is desired.

In this manner papers can be made of which the properties have been changed by functionalization, such as coloring, smoothening, making water repellant, increasing or decreasing the conductivity, and making fire resistant paper.

Because the polymer precursor has been synthesized and spun from solutions that may be free from phosphorus compounds, the PBO obtained can also be free of phosphorus compounds. It is a further advantage that it is no longer required to make the paper from almost insoluble PBO polymers, but the papermaking process can be performed with readily soluble polymer precursors, and conversion to PBO takes place after formation of the paper.

In general the papers from this invention exhibit lower porosity than PPTA papers making them very suitable for electrical applications such as in electrical insulation material. The papers are further suitable for application in honeycomb structures and in constructive materials.

The papers of the present invention, both for PBO precursor-containing papers and PBO papers, have a much higher strength than known papers, as shown by EAB (elongation at break) and TI (tenacity index) data. For instance, the present papers are superior to PPTA paper and even to Nomex®, which is considered the strongest paper known until now.

The extreme strength of the present papers makes it possible to produce extreme thin papers. The papers of this invention also have superior heat stability compared to PPTA paper and Nomex®.

Because of the unusual strength of the present papers, papers having a grammage between 1 and 16 g/m² can be made. The term "grammage" is a metric measure of paper weight based on the same square meter sheet of paper, regardless of paper grade.

The present invention will be explained more specifically by the following embodiments. However, the present invention is not limited to these embodiments.

### General:

These results were obtained with the polymer precursor having the following repeating unit: and with the corresponding ring closed polymer having the repeating unit: wherein Ar¹ = para-phenylene and Ar² = diphenylene

Abbreviations:
NMP = N-methylpyrrolidone
DHB = dihydroxybenzidine (4,4'-diamino-3,3'-dihydroxydiphenyl)
TDC = terephthaloyl dichloride
PPD = para-phenylenediamine
PPTA = para-phenyleneterephthalamide

### Example 1

### Polymerization to polybenzoxazole precursor

2.25 L of NMP/CaCl₂ and 1.75 L of NMP together with pre-dried DHB (140 °C, vacuum, 24 h) were charged into a 10 L Drais reactor and stirred for 30 minutes to let the DHB dissolve. After cooling to 5 °C, TDC was added while continuously stirring (250 rpm). After 50 minutes a sample was taken, 1.8 L of NMP were added. The mixture was stirred for 30 min, another sample was taken and again 1.8 L of NMP were added. The mixture was stirred for 30 min and the reactor was emptied through a bottom valve. By applying this procedure, the first sample had a polymer concentration of 7.4%, the second sample (after dilution with NMP) had a concentration of 5% and the final product had a polymer concentration of 4%. The relative viscosity of the reaction product was 3.43.

The polymerization procedure for the second batch was similar, except that after 60 minutes a sample was taken and 4.0 L of NMP were added. The mixture was stirred for 30 min and then emptied. By applying this procedure, the first sample had a polymer concentration of 7.4% and the final product had a polymer concentration of 4%. The relative viscosity of the reaction product was 3.06.

The polymerization batches were mixed prior to spinning.

### Comparative example 1

Polymerization of PPTA para-phenyleneterephthalamide was carried out using a 160 L Drais reactor. After sufficiently drying the reactor, 64 L of NMP/CaCl₂ with a CaCl₂ concentration of 2.5 wt% were added to the reactor. Subsequently, 1522 g of PPD were added and dissolved at room temperature. Thereafter the PPD solution was cooled to 5 °C and 2824 g of TDC were added. After addition of the TDC the polymerization reaction was continued for 45 min. Then the polymer solution was neutralized with a calcium oxide/NMP-slurry (780 g of CaO in NMP). After addition of the CaO-slurry the polymer solution was stirred for another 30 min. This neutralization was carried out to remove the hydrochloric acid (HCl), which is formed during polymerization. A gel-like polymer solution was obtained with a PPTA content of 4.5 wt% and having a relative viscosity of 3.0 (in 0.25% H₂SO₄).

This product has an etarel (ηᵣₑₗ) of 2.4 and a polymer concentration of 3.6% and was used to spin fibrids as well as pulp. Water was used as coagulant.

### Example 2

### Fibrid and pulp making

The solutions of Example 1 and Comparative Example 1 were spun through a jet spinning nozzle (spinning hole 500 µm) at 20 L/h. Water was added through a ring-shaped channel flowing perpendicular to the polymer flow. During spinning the polymer flow was kept constant while the coagulant pressure was changed for the different samples in order to vary the SR (°SR) of the product.

### Pulp spinning

The solutions of Example 1 and Comparative Example 1 were spun into pulp through a 1 hole jet spinning nozzle (spinning hole 350 µm). The solution was spun into a zone of lower pressure. An air jet was separately applied perpendicularly to the polymer stream through ring-shaped channels to the same zone were expansion of air occurred. Thereafter, the pulp was coagulated with water in the same zone by means of applying a coagulant jet through ring-shaped channels under an angle in the direction of the polymer stream.

To spin the pulp with different SR values (°SR) the air pressure was kept constant while the polymer flow was varied. After spinning all samples were washed with water.

The process and property data of fibrids and pulp obtained in Example 2 are given in Table 1:

**Table 1**

| | | Process parameters | | | | | Properties | | | | |
|---|---|---|---|---|---|---|---|---|---|---|---|
| Sample | Polymer solution | Product type | Polymer solution Flow (L/h) | Coagulant pressure (bar) | Coagulant flow (L/h) | Airflow (Nm³/h) | LL_{0.25} | Fines(%) | SR Value (°SR) | SSA (m²/g) | Dry Solids (%) |
| A | Example1 | pulp | 6 | | 50 | 12 | 0.58 | 43.3 | 63 | 0.6 | 5.3 |
| B | Example1 | fibrid | 20 | 50 | | | 0.72 | 25 | 67 | 0.5 | 7.3 |
| C | CompEx1 | fibrid | 20 | 30 | | | 0.84 | 25 | 42 | 2.2 | 5.6 |
| D | CompEx1 | fibrid | 20 | 50 | | | 0.74 | 26.3 | 65 | 2.6 | 4.8 |
| E | CompEx1 | pulp | 6 | | 50 | 12 | 0.55 | 49.9 | 68 | 5.6 | 7.5 |
| F | CompEx1 | pulp | 18 | | 50 | 12 | 0.62 | 42.7 | 46 | 3.9 | 6.9 |

### Example 3

### Paper making from fibrids

Handsheets from 100% fibrids of samples A1 and B1-B4 and comparative examples D1-D4 and E1 with different grammage were made on a Rapid Kothen machine. The dewatered sheets were dried between two blotting papers under vacuum (95 °C, 1000 mbar, 20 min). Paper data are given in Table 2.

Notice the lower calliper (paper thickness) and higher densities for the papers of the invention in comparison to the reference papers. TI (Tensile Index) is 3-5 times as high for the papers of the invention as for the pulp-based reference papers when compared at the same grammage. EAB is also higher for the papers of the invention.

**Table 2: Properties of paper samples from fibrid**

| Paper Sample | Grammage (g/m²) | Calliper (mm) | Density (g/cm³) | EAB (%) | TI (Nm/g) |
|---|---|---|---|---|---|
| B1 | 99 | 0.168 | 0.59 | 4.3 | 85.2 |
| B2 | 50 | 0.115 | 0.44 | 3.6 | 75.3 |
| B3 | 29 | 0.073 | 0.39 | 3.7 | 72 |
| B4 | 16 | 0.058 | 0.28 | 2.5 | 41.6 |
| D1 | 110 | 0.284 | 0.39 | 1.7 | 28.3 |
| D2 | 52 | 0.193 | 0.27 | 1.7 | 19 |
| D3 | 31 | 0.131 | 0.23 | 1.1 | 14.1 |
| D4 | 16 | 0.092 | 0.17 | 1.6 | 8.1 |

### Example 4

### Paper making from pulp

Handsheets from 100% pulp of samples A and E with a grammage of around 100 g/m² were made on a Rapid Kothen machine using the same procedure as Example 3. Paper data are given in Table 3.

**Table 3: Properties of paper samples from pulp**

| Paper Sample | Grammage (g/m²) | Calliper (mm) | Density (g/cm³) | EAB (%) | TI (Nm/g) |
|---|---|---|---|---|---|
| A1 | 110 | 0.265 | 0.415 | 1.5 | 18.8 |
| E1 | 117 | 0.296 | 0.395 | 1.05 | 9.5 |

### Example 5

### Heat treatment of papers

To convert the above polybenzazole precursor paper to the polybenzazole paper a heat treatment was performed under an inert atmosphere. The procedure was as follows: The samples were enclosed in an oven under a nitrogen flow and heated with a heating rate of 5 °C/min. When the temperature of 440 °C was reached the samples were immediately taken out of the oven. Property data of the samples before and after heat treatment are given in Table 4. IR spectra of the samples were recorded on the Varian FTS-575c infrared spectrometer equipped with the Thunderdome ATR accessory. The spectra confirmed conversion to a polybenzoxazole paper with a conversion factor higher than 95%.

TGA experiments were carried out by means of a Setaram TGA/DSC 111, under nitrogen gas. The paper samples were first cut into pieces and then put in Platinum (open) cells. The sample weight that was used was between 10 and 20 mg. The samples were heated from 20 °C to 700 °C at a heating rate of 10 °C/min.

The onset of degradation Td was determined by the temperature at which 1 weight percent weight loss is found. In case of samples B5 and A1, Td was determined after complete conversion which occurred between 250 and 400 °C. The results are denoted in Table 4.

**Table 4**

| Paper Sample | Type | Heat Treated | Grammage (g/m²) | Calliper (mm) | Density (g/cm³) | Td (°C) | EAB (%) | TI (Nm/g) |
|---|---|---|---|---|---|---|---|---|
| B5 | fibrid paper | No | 102.2 | 0.181 | 0.56 | 631 | 3 | 70 |
| B6 | fibrid paper | Yes | 99.8 | 0.151 | 0.66 | 626 | 3.6 | 80 |
| A1 | pulp paper | No | 110 | 0.265 | 0.42 | 624 | 1.5 | 18.8 |
| A2 | pulp paper | Yes | 118 | 0.207 | 0.57 | 618 | 1.8 | 16.8 |
| D2 | fibrid paper | No | 52 | 0.193 | 0.27 | 540 | 1.7 | 19 |
| D3 | fibrid paper | Yes | 48 | 0.195 | 0.25 | 542 | 1.1 | 9 |

### Example 6

### Making functionalized paper

A precursor paper (paper sample B5), a polybenzoxazole paper obtained by heat treatment of the precursor paper (paper sample B6) and a PPTA paper (paper sample D1) were dyed with a reactive coloring agent (Cibacron Dark Blue S-GL; ex Ciba, Switzerland) according to the following procedure:

A solution of 6 grams of NaCl in 200 mL of demineralized water was prepared at 80 °C. After adding 0.4 g of Cibacron Dark Blue S-GL the solution was stirred for 20 minutes and cooled down to 60 °C. 4.3 grams of Na₂CO₃.10H₂O were added and the solution was stirred for 30 minutes at 60 °C to obtain the dyeing fluid

Samples B5, B6, and D1, each of 5 cm length and 1 cm width, were submerged into the dyeing fluid for 45 minutes at 60 °C and subsequently rinsed in running water of about 50 °C for 10 minutes. The samples were neutralized in a 1% acetic acid bath and washed with running cold water for 15 minutes.

**Table 5: Original color and color after dyeing of the paper samples**

| Paper Sample | Original Color | Color after dyeing |
|---|---|---|
| B5 | light green | dark blue |
| B6 | light brown | light brown |
| D1 | light yellow | light yellow with light blue stains |

The present invention provides aromatic polyamides that are functionalized with a reactive functional group that can be used to facilitate the conjugation of the aramids to a conjugation partner. As shown in Table 5, a functionalized aramid (sample B5) shows excellent dyeability compared to the non-functionalized aramid D1 and to sample B6, which does not contain reactive functional groups due to the complete conversion by heat treatment of B5 to B6, which has a fully ring closed polybenzoxazole structure.

## Claims

1. A paper comprising at least one of a fiber, pulp, fibril, floc, and fibrid having a polybenzazole structure with a repeating unit of formula (I) and/or (II) or its precursor structure with a repeating unit of formula (III): wherein Ar¹ and Ar² are independently a para or meta aromatic group having 4 to 12 carbon atoms, X and Y are the same or different and selected from O, S, and NH; and n is 0 or 1, and wherein the paper is free or essentially free of non-extractable phosphorus compound.

2. The paper of claim 1 obtainable by polymerizing about equimolar amounts of monomers having the formula ClOOC-Ar¹-COOCl and wherein Ar¹ and Ar² are independently a para or meta aromatic group having 4 to 12 carbon atoms, X and Y are the same or different and selected from O, S, and NH; and n is 0 or 1, to the precursor structure containing the repeating unit of formula (III), wherein Ar¹, Ar², X, Y and n have the previously given meanings, optionally followed by cyclising the precursor structure to the polybenzazole structure with the repeating unit of formula (I) and/or (II) wherein Ar¹, Ar², X, and Y have the previously given meanings, in a fluid which is free or essentially free from phosphoric acid.

3. The paper of claim 1 or 2 wherein at least part of XH and/or YH is functionalized.

4. The paper of any one of claims 1-3 having a grammage from 1 to 16 g/m².

5. The paper of any one of claims 1-4 comprising a mixture of at least one of fiber, pulp, fibril, floc, and fibrid having the polybenzazole structure of formula (I) and/or (II), or the polybenzazole precursor structure of formula (III), and PPTA fibrid.

6. A method for making the paper of any one of claims 1 to 5 comprising polymerizing about equimolar amounts of monomers having the formula ClOOC-Ar¹-COOCl and wherein Ar¹ and Ar² are independently a para or meta aromatic group having 4 to 12 carbon atoms, X and Y are the same or different and selected from O, S, and NH; and n is 0 or 1, to a precursor structure containing the repeating unit expressed by formula (III) wherein Ar¹, Ar², X, Y and n have the previously given meanings, optionally followed by cyclising under heating in an inert atmosphere the precursor structure to a polybenzazole structure having a repeating unit of formula (I) and/or (II) wherein Ar¹, Ar², X, and Y have the previously given meanings, in a fluid which is free or essentially free from phosphoric acid, followed by making a fiber, pulp, fibril, floc, or fibrid from the precursor or from the polybenzazole structure, followed by making the paper thereof by a conventional papermaking process optionally followed by one or more of a calendering step, heating step, drying step, and functionalization step.

7. The method according to claim 6 wherein at least part of the XH and/or YH groups of Ar² are functionalized by treating the monomer and/or the precursor structure and/or the polybenzazoe structure with a functionalizing agent.

8. A method for making the paper of any one of claims 1-5 comprising polymerizing about equimolar amounts of monomers having the formula ClOOC-Ar¹-COOCl and wherein Ar¹ and Ar² are independently a para or meta aromatic group having 4 to 12 carbon atoms, X and Y are the same or different and selected from O, S, and NH; and n is 0 or 1, to a precursor having the repeating unit of formula (III) wherein Ar¹, Ar², X, Y and n have the previously given meanings, in a fluid which is free or essentially free from phosphoric acid, followed by making a fiber, pulp, fibril, floc, or fibrid from the precursor, followed by making the paper thereof in a conventional papermaking process, optionally followed by one or more of a calendering step, heating step, drying step, and functionalization step.

9. The method according to claim 7 wherein the paper obtained is heated under an inert atmosphere at a temperature allowing cyclization of the polybenzazole precursor having formula (III) to the polybenzazole comprising the structure of formula (I) and/or (II).

10. The method according to claim 8 or 9 wherein at least part of the XH and/or YH groups of Ar² are functionalized by treating the monomer and/or the precursor structure and/or the polybenzazole structure with a functionalizing agent.

11. A method for making the paper of any one of claims 6 to 10 comprising applying a conventional papermaking process further using at least one of fiber, pulp, fibril, floc, and fibrid having the structure IV wherein the Ar¹ moieties have independently the previously given meaning.

12. An electrical insulation material comprising the paper of any one of claims 1-5.

13. Use of the paper of any one of claims 1-5 for making an electrical insulation material, a honeycomb structure, or a constructive material.

## Patentansprüche

1. Papier, umfassend mindestens eine Faser, Pulpe, Fibrille, Flocke und/oder ein Fibrid, die bzw. das eine Polybenzazol-Struktur mit einer sich wiederholenden Einheit der Formel (I) und/oder (II) aufweist oder dessen Vorläuferstruktur mit einer sich wiederholenden Einheit der Formel (III): wobei Ar¹ und Ar² unabhängig voneinander eine para- oder metaaromatische Gruppe mit 4 bis 12 Kohlenstoffatomen sind, X und Y identisch oder unterschiedlich sind und aus O, S und NH ausgewählt sind; und n gleich 0 oder 1 ist, und wobei das Papier frei oder im Wesentlichen frei von nicht extrahierbaren Phosphorverbindungen ist.

2. Papier nach Anspruch 1, herstellbar durch Polymerisieren ungefähr
equimolarer Mengen von Monomeren mit der Formel ClOOC-Ar¹-COOCl und wobei Ar¹ und Ar² unabhängig voneinander eine para- oder metaaromatische Gruppe mit 4 bis 12 Kohlenstoffatomen sind, X und Y identisch oder unterschiedlich sind und aus O, S und NH ausgewählt sind; und n gleich 0 oder 1 ist, zur Vorläuferstruktur, die die sich wiederholende Einheit der Formel (III) enthält wobei Ar¹, Ar², X, Y und n die zuvor angegebene Bedeutung haben, optional gefolgt von einer Zyklisierung der Vorläuferstruktur zur Polybenzazol-Struktur mit der sich wiederholenden Einheit der Formel (I) und/oder (II) wobei Ar¹, Ar², X und Y die zuvor angegebene Bedeutung haben,
in einem Fluid, das frei oder im Wesentlichen frei von Phosphorsäure ist.

3. Papier nach Anspruch 1 oder 2, bei dem zumindest ein Teil von XH und/oder YH funktionalisiert ist.

4. Papier nach einem der Ansprüche 1 bis 3, das eine flächenbezogene Masse von 1 bis 16 g/m² aufweist.

5. Papier nach einem der Ansprüche 1 bis 4, umfassend ein Gemisch aus mindestens einer Faser, Pulpe, Fibrille, Flocke und/oder einem Fibrid, die bzw. das die Polybenzazol-Struktur mit der Formel (I) und/oder (II) aufweist, oder die Polybenzazol-Vorläuferstruktur mit der Formel (III), und einem PPTA-Fibrid.

6. Verfahren zur Herstellung des Papiers nach einem der Ansprüche 1 bis 5, umfassend das Polymerisieren ungefähr equimolarer Mengen von Monomeren mit der Formel ClOOC-Ar¹-COOCl und wobei Ar¹ und Ar² unabhängig voneinander eine para- oder metaaromatische Gruppe mit 4 bis 12 Kohlenstoffatomen sind, X und Y identisch oder unterschiedlich sind und aus O, S und NH ausgewählt sind; und n gleich 0 oder 1 ist, zu einer Vorläuferstruktur, die die sich wiederholende Einheit enthält, die mit der Formel (III) ausgedrückt wird, wobei Ar¹, Ar², X, Y und n die zuvor angegebene Bedeutung haben, optional gefolgt von einer Zyklisierung der Vorläuferstruktur unter Erhitzung in einer inerten Atmosphäre zu einer Polybenzazol-Struktur, die eine sich wiederholende Einheit der Formel (I) und/oder (II) aufweist wobei Ar¹, Ar², X und Y die zuvor angegebene Bedeutung haben,
in einem Fluid, das frei oder im Wesentlichen frei von Phosphorsäure ist, gefolgt von der Herstellung einer Faser, Pulpe, Fibrille, Flocke oder eines Fibrids aus der Vorläufer- oder aus der Polybenzazol-Struktur, gefolgt von der Herstellung des Papiers daraus mittels eines herkömmlichen Papierherstellungsverfahrens, optional gefolgt von mindestens einem Kalandrierschritt, Erhitzungsschritt, Trocknungsschritt und/oder Funktionalisierungsschritt.

7. Verfahren nach Anspruch 6, wobei zumindest ein Teil der XH- und/oder YH-Gruppen von Ar² durch Behandeln des Monomers und/oder der Vorläuferstruktur und/oder der Polybenzazol-Struktur mit einem Funktionalisierungsmittel funktionalisiert wird.

8. Verfahren zur Herstellung des Papiers nach einem der Ansprüche 1 bis 5, umfassend das Polymerisieren ungefähr equimolarer Mengen von Monomeren mit der Formel ClOOC-Ar¹-COOCl und wobei Ar¹ und Ar² unabhängig voneinander eine para- oder metaaromatische Gruppe mit 4 bis 12 Kohlenstoffatomen sind, X und Y identisch oder unterschiedlich sind und aus O, S und NH ausgewählt sind; und n gleich 0 oder 1 ist, zu einem Vorläufer, der die sich wiederholende Einheit der Formel (III) aufweist wobei Ar¹, Ar², X, Y und n die zuvor angegebene Bedeutung haben, in einem Fluid, das frei oder im Wesentlichen frei von Phosphorsäure ist, gefolgt von der Herstellung einer Faser, Pulpe, Fibrille, Flocke oder eines Fibrids aus dem Vorläufer, gefolgt von der Herstellung des Papiers daraus in einem herkömmlichen Papierherstellungsverfahren, optional gefolgt von mindestens einem Kalandrierschritt, Erhitzungsschritt, Trocknungsschritt und/oder Funktionalisierungsschritt.

9. Verfahren nach Anspruch 7, wobei das hergestellte Papier in einer inerten Atmosphäre bei einer Temperatur erhitzt wird, die die Zyklisierung des Polybenzazol-Vorläufers mit der Formel (III) zum Polybenzazol ermöglicht, das die Struktur mit der Formel (I) und/oder (II) umfasst.

10. Verfahren nach Anspruch 8 oder 9, wobei zumindest ein Teil der XH- und/ oder YH-Gruppen von Ar² durch Behandeln des Monomers und/oder der Vorläuferstruktur und/oder der Polybenzazol-Struktur mit einem Funktionalisierungsmittel funktionalisiert wird.

11. Verfahren zur Herstellung des Papiers nach einem der Ansprüche 6 bis 10, umfassend das Anwenden eines herkömmlichen
Papierherstellungsverfahrens, wobei ferner mindestens eine Faser, Pulpe, Fibrille, Flocke und/oder ein Fibrid mit der Struktur IV verwendet wird, wobei die Ar¹-Anteile unabhängig voneinander die zuvor angegebene Bedeutung haben.

12. Elektrisches Isoliermaterial, welches das Papier nach einem der Ansprüche 1 bis 5 umfasst.

13. Verwendung des Papiers nach einem der Ansprüche 1 bis 5 zur Herstellung eines elektrischen Isoliermaterials, einer Wabenstruktur oder eines Baustoffs.

## Revendications

1. Papier comprenant au moins un élément, parmi des fibres, une pâte, des fibrilles, un floc et des fibrides, qui possède une structure de polybenzazole comportant des motifs répétés de formules (I) et/ou (II) : ou une structure de précurseur d'une telle structure, comportant des motifs répétés de formule (III) : dans lesquelles formules Ar¹ et Ar² représentent, indépendamment, un groupe aromatique de type para ou méta, comportant 4 à 12 atomes de carbone, X et Y représentent des entités identiques ou différentes, choisies parmi celles qui sont symbolisées par O, S et NH, et l'indice n vaut 0 ou 1,
lequel papier ne contient pas ou pratiquement pas de composé phosphoré non extractible.

2. Papier conforme à la revendication 1, qu'on peut obtenir en faisant polymériser, en quantités à peu près équimolaires, des monomères de formules
ClOOC-Ar¹-COOCl et dans lesquelles Ar¹ et Ar² représentent, indépendamment, un groupe aromatique de type para ou méta, comportant 4 à 12 atomes de carbone, X et Y représentent des entités identiques ou différentes, choisies parmi celles qui sont symbolisées par O, S et NH, et l'indice n vaut 0 ou 1,
pour obtenir un précurseur dont la structure comporte des motifs répétés de formule (III) : dans laquelle les symboles Ar¹, Ar², X, Y et n ont les significations indiquées ci-dessus,
et en opérant ensuite, en option, une cyclisation de ce précurseur pour obtenir un polybenzazole dont la structure comporte des motifs répétés de formules (I) et/ou (II) : dans lesquelles les symboles Ar¹, Ar², X et Y ont les significations indiquées ci-dessus,
dans un fluide qui ne contient pas ou pratiquement pas d'acide phosphorique.

3. Papier conforme à la revendication 1 ou 2, dans lequel au moins une partie des groupes symbolisés par XH et/ou YH sont fonctionnalisés.

4. Papier conforme à l'une des revendications 1 à 3, qui présente un grammage de 1 à 16 g/m².

5. Papier conforme à l'une des revendications 1 à 4, comprenant un mélange d'au moins un élément, parmi des fibres, une pâte, des fibrilles, un floc et des fibrides, qui possède une structure de polybenzazole correspondant aux formules (I) et/ou (II) ou une structure de précurseur de polybenzazole correspondant à la formule (III), et de fibrides de poly(para-phénylène-téréphtalamide) (PPTA).

6. Procédé de fabrication d'un papier conforme à l'une des revendications 1 à 5, comportant le fait de faire polymériser, en quantités à peu près équimolaires, des monomères de formules
ClOOC-Ar¹-COOCl et dans lesquelles Ar¹ et Ar² représentent, indépendamment, un groupe aromatique de type para ou méta, comportant 4 à 12 atomes de carbone, X et Y représentent des entités identiques ou différentes, choisies parmi celles qui sont symbolisées par O, S et NH, et l'indice n vaut 0 ou 1,
pour obtenir un précurseur dont la structure comporte des motifs répétés de formule (III) : dans laquelle les symboles Ar¹, Ar², X, Y et n ont les significations indiquées ci-dessus,
et le fait de faire ensuite, en option, cycliser ce précurseur, à chaud et dans une atmosphère inerte, pour obtenir un polybenzazole dont la structure comporte des motifs répétés de formules (I) et/ou (II) : dans lesquelles les symboles Ar¹, Ar², X et Y ont les significations indiquées ci-dessus,
dans un fluide qui ne contient pas ou pratiquement pas d'acide phosphorique, puis le fait de mettre le précurseur ou le polybenzazole sous une forme de fibres, de pâte, de fibrilles, de floc ou de fibrides, d'en faire un papier suivant un procédé classique de fabrication de papier, et d'opérer ensuite, en option, une ou plusieurs étapes parmi une étape de calandrage, une étape de chauffage, une étape de séchage et une étape de fonctionnalisation.

7. Procédé conforme à la revendication 6, dans lequel au moins une partie des groupes XH et/ou YH liés au groupe Ar² sont fonctionnalisés par traitement du monomère et/ou du précurseur et/ou du polybenzazole avec un agent de fonctionnalisation.

8. Procédé de fabrication d'un papier conforme à l'une des revendications 1 à 5, comportant le fait de faire polymériser, en quantités à peu près équimolaires, des monomères de formules
ClOOC-Ar¹-COOCl et dans lesquelles Ar¹ et Ar² représentent, indépendamment, un groupe aromatique de type para ou méta, comportant 4 à 12 atomes de carbone, X et Y représentent des entités identiques ou différentes, choisies parmi celles qui sont symbolisées par O, S et NH, et l'indice n vaut 0 ou 1,
pour obtenir un précurseur comportant des motifs répétés de formule (III) : dans laquelle les symboles Ar¹, Ar², X, Y et n ont les significations indiquées ci-dessus,
dans un fluide qui ne contient pas ou pratiquement pas d'acide phosphorique, et le fait de mettre ce précurseur sous une forme de fibres, de pâte, de fibrilles, de floc ou de fibrides, d'en faire un papier suivant un procédé classique de fabrication de papier, et d'effectuer ensuite, en option, une ou plusieurs étapes parmi une étape de calandrage, une étape de chauffage, une étape de séchage et une étape de fonctionnalisation.

9. Procédé conforme à la revendication 7, dans lequel le papier obtenu est chauffé sous atmosphère inerte à une température qui permet que se déroule une cyclisation du précurseur de polybenzazole de formule (III) en un polybenzazole comportant des motifs de formules (I) et/ou (II).

10. Procédé conforme à la revendication 8 ou 9, dans lequel au moins une partie des groupes XH et/ou YH liés au groupe Ar² sont fonctionnalisés par traitement du monomère et/ou du précurseur et/ou du polybenzazole avec un agent de fonctionnalisation.

11. Procédé de fabrication de papier, conforme à l'une des revendications 6 à 10, qui comporte le fait de mettre en oeuvre un procédé classique de fabrication de papier, en utilisant en outre au moins un élément, parmi des fibres, une pâte, des fibrilles, un floc et des fibrides, qui possède des motifs de structure (IV) : dans laquelle les symboles Ar¹ ont, indépendamment, les significations indiquées plus haut.

12. Matériau d'isolation électrique, comprenant un papier conforme à l'une des revendications 1 à 5.

13. Utilisation d'un papier conforme à l'une des revendications 1 à 5 pour la fabrication d'un matériau d'isolation électrique, d'une structure en nid d'abeilles ou d'un matériau de construction.
